

## UNITED STATES PATENT OFFICE

2,689,849

CYANINE DYES CONTAINING THE TRI-AZOLO[4,3- $\alpha$ ]QUINOLINE OR TETRA-AZOLO[ $\alpha$ ]QUINOLINE NUCLEUSLeslie G. S. Brooker, Rochester, N. Y., assignor to  
Eastman Kodak Company, Rochester, N. Y., a  
corporation of New JerseyNo Drawing. Application September 10, 1952,  
Serial No. 308,908

10 Claims. (Cl. 260—240.6)

1

The instant application relates to new cyanine dyes, useful in sensitizing photographic halide emulsions, and methods for making such dyes.

Certain dyes of the cyanine dye series are known to extend the sensitivity of photographic silver halide emulsions. Dyes which have been found useful for this purpose include those which contain a quinoline nucleus. Such dyes have been long known, although they have not been particularly efficacious for such purposes as sensitizers for photographic emulsions. While dyes of the above mentioned type are classed as weak sensitizers, I have now found a new class of dyes, some of which are especially useful in extending the sensitivity of photographic silver halide emulsions.

It is an object of the present invention to provide new dyes of the cyanine series and to provide a process for preparing such dyes. A further object is to provide photographic silver halide emulsions sensitized with such dyes. A still further object is to provide a process for preparing photographic silver halide emulsions containing these new dyes. Other objects will become apparent hereinafter.

The new dyes of the cyanine series of my invention can be represented by the following general formula:



wherein R and R<sub>1</sub> each represents an alkyl group, such as methyl, ethyl, n-propyl, isopropyl, n-butyl, benzyl (phenylmethyl), etc., D represents the non-metallic atoms necessary to complete a carbocyclic nucleus of the benzene series, X represents an acid radical, such as chloride, bromide, iodide, perchlorate, thiocyanate, benzenesulfonate, p-toluenesulfonate, ethylsulfate, methylsulfate, etc., Q represents a nitrogen atom or a methine group, d and n each represents a positive integer of from 1 to 2, and Z represents the non-metallic atoms necessary to complete a heterocyclic nucleus containing from five to six atoms in the heterocyclic ring, such as those selected from the group consisting of those of the thiazole series (e. g. thiazole, 4-methylthiazole, 4-phenylthiazole, 5-methylthiazole, 5-phenylthiazole, 4,5-dimethylthiazole, 4,5-diphenylthiazole, 4-(2-thienyl)thiazole, etc.), those of the benzo-

2

thiazole series (e. g. benzothiazole, 4-chlorobenzothiazole, 5-chlorobenzothiazole, 6-chlorobenzothiazole, 7-chlorobenzothiazole, 4-methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 5-iodobenzothiazole, 6-iodobenzothiazole, 4-ethoxybenzothiazole, 5-ethoxybenzothiazole, tetrahydrobenzothiazole, 5,6-dimethoxybenzothiazole, 5,6-dioxymethylenebenzothiazole, 5-hydroxybenzothiazole, 6-hydroxybenzothiazole, etc.), those of the naphthothiazole series (e. g.  $\alpha$ -naphthothiazole,  $\beta$ -naphthothiazole, 5-methoxy- $\beta$ -naphthothiazole, 8-methoxy- $\alpha$ -naphthothiazole, 7-methoxy- $\alpha$ -naphthothiazole, etc.), those of the thianaphtheno-7',6',4,5-thiazole series (e. g. 4'-methoxythianaphtheno-7',6',4,5-thiazole, etc.), those of the oxazole series (e. g. 4-methyloxazole, 5-methyloxazole, 4-phenyloxazole, 4,5-diphenyloxazole, 4-ethyloxazole, 4,5-dimethyloxazole, 5-phenyloxazole, etc.), those of the benzoxazole series (e. g. benzoxazole, 5-chlorobenzoxazole, 5-methylbenzoxazole, 5-phenylbenzoxazole, 6-methylbenzoxazole, 5,6-dimethylbenzoxazole, 4,6-dimethylbenzoxazole, 5-methoxybenzoxazole, 5-ethoxybenzoxazole, 5-chlorobenzoxazole, 6-methoxybenzoxazole, 5-hydroxybenzoxazole, 6-hydroxybenzoxazole, etc.), those of the naphthoxazole series (e. g.  $\alpha$ -naphthoxazole,  $\beta$ -naphthoxazole, etc.), those of the selenazole series (e. g. 4-methylselenazole, 4-phenylselenazole, etc.), those of the benzoselenazole series (e. g. benzoselenazole, 5-chlorobenzoselenazole, 5-methoxybenzoselenazole, 5-hydroxybenzoselenazole, tetrahydrobenzoselenazole, etc.), those of the naphthoselenazole series (e. g.  $\alpha$ -naphthoselenazole,  $\beta$ -naphthoselenazole, etc.), those of the thiazoline series (e. g. thiazoline, 4-methylthiazoline, etc.), those of the 2-quinoline series (e. g. quinoline, 3-methylquinoline, 5-methylquinoline, 7-methylquinoline, 8-methylquinoline, 6-chloroquinoline, 8-chloroquinoline, 6-methoxyquinoline, 6-ethoxyquinoline, 6-hydroxyquinoline, 8-hydroxyquinoline, etc.), those of the 4-quinoline series (e. g. quinoline, 6-methoxyquinoline, 7-methylquinoline, 8-methylquinoline, etc.), those of the 1-isoquinoline series (e. g. isoquinoline, 3,4-dihydroisoquinoline, etc.), those of the 3-isoquinoline series (e. g. isoquinoline, etc.), those of the 3,3-dialkylindolenine series (e. g. 3,3-dimethylindolenine, 3,3,5-trimethylindolenine, 3,3,7-trimethylindolenine, etc.), the pyridine series (e. g. pyridine, 5-methylpyridine, etc.), etc.

The cyanine dyes represented by Formula I above ( $d$  is 1) can advantageously be prepared by condensing a cyclammonium quaternary salt selected from those represented by the following general formula:

II



wherein R, D, Q and X each have the values set forth above, together with a cyclammonium quaternary salt selected from those represented by the following general formula:

III



wherein R<sub>1</sub>, n, and Z each have the values given above, X<sub>1</sub> represents an acid radical, e. g. chloride, bromide, iodide, perchlorate, thiocyanate, benzenesulfonate, p-toluenesulfonate, ethylsulfate, methylsulfate, etc., and R<sub>2</sub> represents an alkyl group, e. g. methyl, ethyl, etc., or an aryl group, e. g. phenyl, tolyl (o-, m-, and p-), etc. The condensations can advantageously be carried out in the presence of a basic condensing agent, e. g. the organic tertiary amines, such as triethylamine, tri-n-propylamine, triisopropylamine, tri-n-butylamine, etc., N-methylpiperidine, N-ethylpiperidine, N,N-dimethylaniline, N,N-diethylaniline, etc. The condensations can advantageously be effected in the presence of an inert solvent, e. g. ethanol, isopropanol, 1,4-dioxane, etc. Heating accelerates the condensations and temperatures varying from room temperature (about 20° C.) to the temperature of the steam bath can be used.

The cyclammonium quaternary salts selected from those represented by Formula II above can advantageously be prepared by heating the corresponding free base together with an alkyl salt, e. g.

R-X

wherein R and X each have the values given above. The free bases can be prepared in accordance with the method described by Marckwald et al. in "Berichte" (1900), volume 33, pages 1885-1899. Quaternization can be effected by simply heating the free base together with the alkyl salt on an oil bath or a steam bath until the mass sets to a solid (generally 10-20 hours). The cyclammonium quaternary salts can have substituents on the carbocyclic ring, such as halogen (e. g. chlorine, bromine, etc.), hydroxyl, alkoxy, etc.

The carbocyanine dyes represented by Formula I above ( $d$  is 2) can advantageously be prepared by condensing a cyclammonium quaternary salt selected from those represented by the following general formula:

IV



wherein R<sub>1</sub>, X<sub>1</sub>, n, and Z each have the values given above, R<sub>3</sub> represents an acyl group (e. g. acetyl, propionyl, benzoyl, etc.), and R<sub>4</sub> repre-

sents an aromatic group (e. g. phenyl, tolyl, naphthyl, etc.), together with a cyclammonium quaternary salt selected from those represented by Formula II above. The condensations can advantageously be effected in the presence of a basic condensing agent, such as those set forth above for the condensation of the compounds of Formula II with those of Formula III. Likewise, the condensations can advantageously be effected in the presence of an inert solvent, such as those set forth above for the condensation of the compounds of Formula II with those of Formula III. Heating accelerates the condensations and temperatures varying from room temperature (about 20° C.) to the temperature of the steam bath can be used. The following examples will serve to illustrate more fully the manner whereby I practice my invention.

20 Example 1.—1',3-diethyl-5-s-triazolo[4,3-a]-quino-2'-cyanine perchlorate



25 0.87 gram (1 mol.) of 5-methyl-3-triazolo[4,3-a]quinoline and 1.50 grams (1 mol.+50% excess) of ethyl p-toluenesulfonate were heated together on an oil bath at 140° C. for 15 hours. After cooling the fused mass to room temperature, 1.97 grams (1 mol.) of 2-phenylmercaptoquinoline ethiodide, 1.11 grams (2 mols.+5% excess) of triethylamine and 13 cc. of pyridine were then added and the resulting mixture refluxed 40 25 minutes. After precipitating the dye with an excess of aqueous potassium perchlorate, it was chilled, filtered off, washed well with hot water and acetone and crystallized twice from methyl alcohol; (160 cc./gram). The final yield was 13% of the theoretical. The maroon crystals melted at 217-218° C. dec.

45 Example 2.—3,3'-diethylthia-5'-s-triazolo[4,3-a]quinocyanine perchlorate



50 60 0.87 gram (1 mol.) of 5-methyl-s-triazolo[4,3-a]quinoline and 1.50 grams (1 mol.+50% excess) of ethyl p-toluenesulfonate were heated together on an oil bath at 140° C. for 15 hours. After cooling the fused mass to room temperature, 2.00 grams (1 mol.) of 2-phenylmercaptobenzothiazole ethiodide, 1.11 grams (2 mols.+5% excess) of triethylamine and 15 cc. of pyridine were then added and the resulting mixture refluxed 25 minutes. After precipitating the dye with an excess of aqueous potassium perchlorate, it was chilled, filtered off, washed with hot water and acetone and crystallized twice from methyl alcohol; (340 cc./gram). The final yield was 15% of the theoretical. The felt-like mass of 65 70 orange crystals melted at 255-257° C. dec.

*Example 3.—3,3'-diethylthia-5'-s-triazolo[4,3-a]quinocarbocyanine perchlorate*



0.87 gram (1 mol.) of 5-methyl-s-triazolo[4,3-a]quinoline and 1.50 grams (1 mol.+50% excess) of ethyl p-toluenesulfonate were heated together on an oil bath at 140° C. for 15 hours. After cooling the fused mass to room temperature, 2.25 grams (1 mol.) of 2-β-acetanilidovinylbenzothiazole ethiodide, 1.11 grams (2 mols.+5% excess) of triethylamine and 15 cc. of pyridine were then added and the resulting mixture refluxed for 30 minutes. After precipitating the dye with an excess of aqueous potassium perchlorate, it was chilled, filtered off, washed well with hot water and acetone and crystallized twice from methyl alcohol; (330 cc./gram). The final yield was 8%. The purplish crystalline powder melted at 236-238° C. dec.

*Example 4.—3,3'-diethyl-5-tetrazolo[a]-quinothiacyanine iodide*



0.92 gram (1 mol.) of 5-methyltetrazolo[4,3-a]quinoline and 1.50 grams (1 mol.+50% excess) of ethyl p-toluenesulfonate were heated together on an oil bath at 140° C. for 15 hours. After cooling the fused mass to room temperature, 2.00 grams (1 mol.) of 2-phenylmercaptobenzothiazole ethiodide, 1.11 grams (2 mols.+5% excess) of triethylamine and 15 cc. of ethyl alcohol were then added and the resulting mixture refluxed 15 minutes and then chilled. The crude dye that separated was filtered off, washed with cold ethyl alcohol, water, acetone and then crystallized twice from methyl alcohol; (150 cc./gram). The final yield was 11% of the theoretical. The orange crystals melted at 245-247° C. dec.

*Example 5.—1',3-diethyl-5-tetrazolo[a]-quino-2'-cyanine iodide*



0.92 gram (1 mol.) of 5-methyltetrazolo[4,3-a]quinoline and 1.50 grams (1 mol.+50% excess) of ethyl p-toluenesulfonate were heated together on an oil bath at 140° C. for 15 hours. After cooling the fused mass to room temperature, 1.97 grams (1 mol.) of 2-phenylmercaptquinoline ethiodide, 1.11 grams (2 mols.+5% excess) of triethylamine and 15 cc. of ethyl alcohol were then added and the resulting mixture refluxed 15 minutes and then chilled. The crude dye was filtered off, washed with cold ethyl alcohol, water, acetone and then crystallized twice from methyl alcohol; (57 cc./gram). The final yield was 31% of the

theoretical. The brilliant copper flakes melted at 244-246° C. dec.

*Example 6.—3,3'-diethyloxa-5'-tetrazolo[a]-quinocarbocyanine iodide*



0.92 gram (1 mol.) of 5-methyltetrazolo[4,3-a]quinoline and 1.50 grams (1 mol.+50% excess) of ethyl p-toluenesulfonate were heated together on an oil bath at 140° C. for 15 hours. After cooling the fused mass to room temperature, 2.17 grams (1 mol.) of 2-β-acetanilidovinylbenzoxazole ethiodide, 1.11 grams (2 mols.+5% excess) of triethylamine and 15 cc. of ethyl alcohol were then added and the resulting mixture refluxed 15 minutes and then chilled. The crude dye that separated was filtered off, washed with cold ethyl alcohol, water, acetone and then crystallized twice from methyl alcohol; (59 cc./gram). The final yield was 35% of the theoretical. The bluish-green needles melted at 234-236° C. dec.

*Example 7.—3'-ethyl-3-methyl-5-tetrazolo[a]-quinothiacyanine p-toluenesulfonate*



0.92 gram (1 mol.) of 5-methyltetrazolo[4,3-a]quinoline and 1 gram (1 mol.+7% excess) of methyl-p-toluenesulfonate were heated together for 20 hours on a steam bath. The melt was cooled and washed with ether. 1.75 grams (1 mol.) of 2-ethylmercaptobenzothiazole ethoethylsulfate, 15 cc. of ethyl alcohol, and 1.1 grams (2 mols.+10% excess) of triethylamine were added to the crude quaternary salt, and the mixture was refluxed for 30 minutes. The reaction mixture was cooled and treated with ether. The residue was titrated with ethyl alcohol, and the dye was filtered off and washed with ethyl alcohol. After two recrystallizations from methyl alcohol (650 cc./gram) the yield was 5% of the theoretical. The orange crystals melted at 255-256° C. dec.

It has also been found that the intermediates represented by Formula II above can be condensed with a p-aminoaromatic aldehyde to produce dyes of the styryl class. Useful aldehydes include, for example, p-dimethylaminobenzaldehyde, p-diethylaminobenzaldehyde, etc. The condensations are advantageously effected in the presence of a basic condensing agent, e. g. piperidine, etc. The condensations can be carried out in the presence of an inert solvent, e. g., ethanol, propanol, isopropanol, n-butanol, etc. Heating accelerates the condensations and temperatures varying from room temperature (about 20° C.) to the temperature of the steam bath can be used. The styryl dyes thus obtained have been found to be particularly useful in the preparation of filter layers, overcoating layers, and the like in photographic elements.

The following examples will serve to illustrate the manner whereby styryl dyes can be prepared according to my invention.

*Example 8.—5-dimethylaminostyryl-3-ethyl-8-triazolo[4,3-a]quinolinium iodide*



1.73 grams (1 mol.) of 5-methyl-s-triazolo [4,3-a] quinoline and 4 grams (1 mol.+100% excess) of ethyl-p-toluenesulfonate were heated together for 20 hours on a steam bath. The melt was cooled to room temperature and washed with ether. 1.5 grams (1 mol.) of p-dimethylaminobenzaldehyde and 5 cc. of piperidine were added to the crude quaternary salt and the mixture was refluxed for five minutes. The reaction mixture was cooled and extracted twice with ether. The residue was dissolved in ethyl alcohol and treated with an aqueous solution of sodium iodide. After cooling, the crystals were filtered off and washed with ethyl alcohol. After two recrystallizations from methyl alcohol (100 cc./gram) the yield was 17% of the theoretical. The reddish-brown crystals melted at 278-280° C. dec.

*Example 9.—5-p-dimethylaminostyryl - 3 - ethyl-tetrazolo [a] quinolinium iodide*



0.92 gram (1 mol.) of 5-methyltetrazolo [a] quinoline and 1.50 grams (1 mol.+50% excess) of ethyl p-toluenesulfonate were heated together on an oil bath at 140° C. for 15 hours. After cooling the fused mass to room temperature, 1.49 grams (2 mols.) of p-dimethylaminobenzaldehyde, 0.47 grams (1 mol.+10% excess) of piperidine and 15 cc. of ethyl alcohol were added and the mixture refluxed 40 minutes. After precipitating the dye with an excess of aqueous potassium iodide, it was then chilled, filtered off, washed with ethyl alcohol, water, acetone and crystallized twice from methyl alcohol; (200 cc./gram). The final yield was 50% of the theoretical. The maroon needles melted at 259-261° C. dec.

As shown above I have found that my new cyanine dyes (Formula I) spectrally sensitize photographic silver halide emulsions when incorporated therein. The dyes are especially useful for extending the spectral sensitivity of the customarily employed gelatino-silver-chloride, gelatino-silver-chlorobromide, gelatino - silver - bromide and gelatino-silver-bromiodide developing-out emulsions. To prepare emulsions sensitized with one or more of my new dyes, it is only necessary to disperse the dye or dyes in the emulsions. The methods of incorporating dyes in emulsions are simple and are known to those skilled in the art. In practice, it is convenient to add the dyes to the emulsions in the form of a solution in an appropriate solvent. Methanol or acetone has proved satisfactory as a solvent for most of my new cyanine dyes. Where the dyes are quite insoluble in methyl alcohol, a mixture of acetone and pyridine is advantageously employed as a solvent. The dyes are advantageously incorporated in the finished, washed emulsions and should be uniformly distributed throughout the emulsions. The particular solvent used will, of

course, depend on the solubility properties of the particular dye.

The concentration of the dyes in the emulsions can vary widely, e. g. from 5 to 100 mg. per liter of flowable emulsion. The concentration of the dyes will vary according to the type of emulsion and according to the effect desired. The suitable and most economical concentration for any given emulsion will be apparent to those skilled in the art, upon making the ordinary tests and observations customarily used in the art of emulsion making. To prepare a gelatino-silver-halide emulsion sensitized with one or more of my new dyes, the following procedure is satisfactory.

15 A quantity of dye is dissolved in methyl alcohol or acetone (or a mixture of acetone and pyridine) and a volume of this solution, which may be diluted with water, containing from 5 to 100 mg. of dye, is slowly added to about 1000 cc. of gelatino-silver-halide emulsion, with stirring. Stirring is continued until the dye is thoroughly dispersed in the emulsion.

20 With most of my dyes, from 10 to 20 mg. of dye per liter of gelatino-silver-bromide or bromo-iodide emulsion (containing about 40 g. of silver halide) suffices to produce the maximum sensitizing effect. With the finer grain emulsions, somewhat larger concentrations of dye may be needed to produce the maximum sensitizing effect.

25 The above statements are only illustrative, as it will be apparent that the dyes can be incorporated in photographic emulsions by any of the other methods customarily employed in the art, e. g. by bathing a plate or film upon which an emulsion is coated in a solution of the dye in an appropriate solvent. However, bathing methods are ordinarily not to be preferred. Emulsions sensitized with the dyes can be coated on suitable supports, such as glass, cellulose derivative film, resin film or paper in the usual manner.

30 For the preparation of overcoating layers, filter layers, antihalation layers, etc., from the styryl dyes obtained according to my invention, from 50 mg. to 150 mg. of styryl dye is dissolved in from 2 to 5 cc. of water-miscible solvent. Methanol or acetone is suitable for this purpose, but pyridine or  $\beta$ -ethoxyethanol can also be used. The solution is then added to about 25 cc. of a 5% gelatin solution at about 40° C. and the mixture coated on the support.

35 It has also been found that a 2-alkylmercaptolepidine selected from those represented by the following general formula:

V



40 wherein  $R_5$  represents an alkyl group, e. g. methyl, ethyl, etc., can be heated with an alkyl salt ( $R_6-X_2$ ) to give a quaternary salt having the following general formula:

V(a)



45 wherein  $R_5$  has the values given above,  $R_6$  represents an alkyl group, e. g. methyl, ethyl, etc., and  $X_2$  represents an acid radical, e. g. chloride, bromide, iodide, p-toluenesulfonate, etc.

The intermediates represented by Formula V (a) above can be condensed with a compound selected from those represented by Formula IV above to give a carbocyanine dye selected from those represented by the following general formula:

VI



wherein  $R_1$ ,  $R_5$ ,  $R_6$ ,  $X_2$ ,  $n$ , and  $Z$  each have the values given above. These dyes, likewise, have been found useful for altering the sensitivity of photographic silver halide emulsions. The condensations can advantageously be effected in the presence of a basic condensing agent, e. g. triethylamine, tri-n-butylamine, etc. Inert solvents can also be employed in the condensations, such solvents as ethanol, n-butanol, etc., being particularly useful. Heating accelerates the condensations and temperature varying from room temperature (about 20° C.) to the reflux temperature of the reaction mixture can be employed.

It has been found that the carbocyanine dyes selected from those represented by Formula VI above can be treated with sodium sulfide or sodium selenide to produce un-ionized dyes represented by the following resonance structures:

VII



wherein  $R_1$ ,  $R_6$ ,  $n$  and  $Z$  each have the values given above. The dyes represented by Formula VII above give colors in solution that are considerably deepened on adding a solution of silver nitrate, indicating the formation of the isomer represented as Formula VII (b) above. Such dyes are, accordingly, excellent indicators for the presence of the silver ion. Some of the new dyes represented by Formula VII are also useful in extending the sensitivity of photographic silver halide emulsions.

The following examples will serve to illustrate the manner whereby the new dyes represented by Formulas VI and VII can be prepared according to my invention.

*Example 10.—1',3-diethyl-2'-ethylmercapto-oxa-4'-carbocyanine perchlorate*



12.0 grams (1 mol.) of 2-ethylmercaptolepidine ethoethylsulfate, 16.0 grams (1 mol.) of 2- $\beta$ -acetanilidovinylbenzoxazole ethiodide, 8.2 grams (2 mols. +10% excess) of triethylamine and 70

5 cc. of ethyl alcohol were refluxed for 12 minutes and the dye precipitated with an excess of aqueous potassium perchlorate. After chilling the reaction mixture, the dye was filtered off, washed with cold ethyl alcohol, hot water, acetone and crystallized twice from methyl alcohol; (500 cc./gram). The final yield was 25% of the theoretical. The minute green crystals melted at 251–253° C. dec.

*Example 11.—1',3-diethyl-2'-ethylmercaptothia-4'-carbocyanine perchlorate*



12.0 grams (1 mol.) of 2-ethylmercaptolepidine ethoethylsulfate, 16.6 grams (1 mol.) of 2- $\beta$ -acetanilidovinylbenzothiazole ethiodide, 8.2 grams (2 mols. +10% excess) of triethylamine and 75 cc. of ethyl alcohol were mixed and refluxed 20 minutes and the dye precipitated with an excess of aqueous potassium perchlorate. After chilling the reaction mixture, the dye was filtered off, washed with cold ethyl alcohol, hot water, acetone and crystallized twice from methyl alcohol; (400 cc./gram). The minute bronze crystals melted at 251–253° C. dec.

*Example 12.—1-ethyl-4-(3-ethyl-2(3H)-benzoxazolylidene) propenylthiocarbostyryl*



12.5 grams (1 mol.) of 1',3-diethyl-2'-ethylmercapto-oxa-4'-carbocyanine perchlorate, 0.98 gram (1 mol. +25% excess) of anhydrous sodium sulfide and 30 cc. of absolute ethyl alcohol were refluxed 10 minutes during which time the deep blue color of the reaction mixture reverted to a dull orange. After chilling several hours at 0° C., the green crystals were filtered off, washed with a few cc. of cold methyl alcohol and crystallized twice from ethyl alcohol; (250 cc./gram). The long maroon needles melted at 207–209° C. dec.

*Example 13.—1-ethyl-4-(3-ethyl-2(3H)-benzothiazolylidene) propenylthiocarbostyryl*



2.60 grams (1 mol.) of 1'-3-diethyl-2'-ethylmercaptothia-4'-carbocyanine perchlorate, 0.98 gram (1 mol. +25% excess) of anhydrous sodium sulfide and 30 cc. of anhydrous ethyl alcohol were refluxed 5 minutes during which time the deep blue color of the reaction mixture was replaced by a reddish coloration. After chilling several hours at 0° C., the green crystals were filtered off, washed with a few cc. of cold ethyl alcohol,

11

then a large quantity of hot water and cold methyl alcohol. The dye was purified by dissolving in pyridine and precipitating with methyl alcohol. The minute green crystals melted at 243-246° C. dec.

The above examples are merely illustrative, and it is to be understood that various modifications can be made in accordance with the general description given above.

What I claim as my invention and desire secured by Letters Patent of the United States is:

1. A cyanine dye selected from those represented by the following general formula:



wherein R and R<sub>1</sub> each represents an alkyl group containing from 1 to 4 carbon atoms, d and n each represents a positive integer of from 1 to 2, Q represents a member selected from the group consisting of a nitrogen atom and a —CH=group, X represents an acid radical, and Z represents the non-metallic atoms necessary to complete a heterocyclic nucleus selected from the group consisting of those of the thiazole series, those of the benzothiazole series, those of the naphthothiazole series, those of the thianaphtheno-7',6',4,5-thiazole series, those of the oxazole series, those of the benzoxazole series, those of the naphthoxazole series, those of the selenazole series, those of the benzoselenazole series, those of the naphthoselenazole series, those of the thiazoline series, those of the 2-quinoline series, those of the 4-quinoline series, those of the 1-isoquinoline series, those of the 3-isoquinoline series, those of the 3,3-dialkyl-indolene series, and those of the pyridine series.

2. A cyanine dye selected from those represented by the following general formula:



wherein R and R<sub>1</sub> each represents an alkyl group containing from 1 to 4 carbon atoms, d and n each represents a positive integer of from 1 to 2, X represents an acid radical, and Z represents the non-metallic atoms necessary to complete a heterocyclic nucleus containing from 5 to 6 atoms in the heterocyclic ring.

3. The cyanine dye having the following formula:



12

4. The cyanine dye having the following formula:



5. The cyanine dye having the following formula:



6. The cyanine dye having the following formula:



7. The cyanine dye having the following formula:



8. A process for preparing cyanine dyes comprising condensing together a compound selected from those represented by the following general formula:



wherein R represents an alkyl group containing from 1 to 4 carbon atoms, Q represents a member selected from the group consisting of a nitrogen atom and a —CH=group, and X represents an acid radical, and a compound selected from those represented by the following two general formulas:



and



wherein R<sub>1</sub> represents an alkyl group containing from 1 to 4 carbon atoms, R<sub>2</sub> represents a member selected from the group consisting of an alkyl group containing from 1 to 2 carbon atoms, a

13

phenyl group, and a tolyl group,  $R_3$  represents an acyl group of a carboxylic acid,  $R_4$  represents a mononuclear aromatic group,  $n$  represents a positive integer of from 1 to 2,  $X_1$  represents an acid radical, and  $Z$  represents the non-metallic atoms necessary to complete a heterocyclic nucleus selected from the group consisting of those of the thiazole series, those of the benzothiazole series, those of the naphthothiazole series, those of the oxazole series, those of benzoxazole series, those of the naphthoxazole series, those of the selenazole series, those of the benzoselenazole series, those of the naphthoselenazole series, those of the thiazoline series, those of the thianaphtheno-7',6',4,5-thiazole series, those of the 2-quinoline 15

14

series, those of the 4-quinoline series, those of the 1-isoquinoline series, those of the 3-isoquinoline series, those of the 3,3-dialkyldolene series, and those of the pyridine series.

5 9. A process according to claim 8 wherein the condensation is carried out in the presence of a basic condensing agent.

10 10. A process according to claim 9 wherein the basic condensing agent is triethylamine.

References Cited in the file of this patent

UNITED STATES PATENTS

| Number    | Name     | Date         |
|-----------|----------|--------------|
| 2,443,136 | Heimbach | June 8, 1948 |